

## UNITED STATES PATENT OFFICE

2,682,461

## SOLID GAS GENERATING CHARGE

Alexander C. Hutchison, Saltcoats, Scotland, assignor to Imperial Chemical Industries Limited, a corporation of Great Britain

No Drawing. Application November 18, 1949,  
Serial No. 128,240

Claims priority, application Great Britain  
January 12, 1949

4 Claims. (Cl. 52—5)

1

The present invention relates to improvements in solid gas-generating charges of the kind capable of propagating through themselves a self-sustaining exothermic non-detonating gas-evolving decomposition when a merely local portion of the charge is heated from room temperature to the temperature at which its active decomposition begins. Such gas-generating charges have found application for a variety of purposes including, for instances, the actuation of gas pressure operated mechanical devices, blasting operations, the dispersion of volatilizable pesticides, insect repellants, rodenticides, propulsion of rockets and the expulsion of liquids from containers such as fire extinguishers.

It is known that guanidine nitrate undergoes an exothermic gas-evolving decomposition when it is strongly heated, but under atmospheric pressure conditions the reaction does not sustain itself if a portion only of a quantity of the compound is heated from atmospheric temperature to the temperature at which decomposition begins, unless external heating is maintained. The decomposition leads to the production of gases which include steam, nitrogen, ammonia and oxides of carbon, but there is also formed a certain amount of a difficultly fusible-yellow nitrogenous organic residue.

When the conditions are such that the prevailing gas pressure is sufficiently high, namely of the order of 70 atmospheres, once the reaction has been locally initiated it will sustain itself throughout a mass of the guanidine nitrate.

It has been proposed to provide charges capable of decomposing in a self-sustained manner with a high yield of permanent gases when locally heated by a non-detonating element, at a lower pressure than guanidine nitrate, said mixtures comprising guanidine nitrate with a proportion of a metallic hypophosphite or ammonium hypophosphite whereby, if desired, charges capable of supporting their decomposition even at atmospheric pressure when locally heated may be obtained.

Owing to the nature or amount of the residue the hypophosphites leave behind or other disadvantages attendant on their employment, these charges have a limited applicability and it would be desirable to provide improved gas-generating charges based on guanidine nitrate and capable of self-sustained decomposition under conditions of much lower gas pressure than guanidine nitrate alone.

It is also known that the pressure required to render possible the self-sustained decomposition of a charge based on guanidine nitrate may be

progressively reduced by making up the guanidine nitrate into charges with progressively increasing amounts of colloided nitrocellulose as a binding agent, by mixing the guanidine nitrate with a solution of nitrocellulose in a volatile solvent, forming the resulting paste into the required shape and evaporating off the volatile solvent, but the use of a volatile solvent adds to the expense and necessitates a drying operation, while the applicability of this method is also somewhat limited.

In British patent specification No. 627,724 there is claimed inter alia gas-producing charges comprising nitroguanidine and/or guanidine nitrate and a pulverulent metal, non-metal or metallic compound sensitiser other than a metallic hypophosphite or ammonium hypophosphite, for the thermal decomposition of nitroguanidine and/or guanidine nitrate.

In co-pending British specification No. 644,073 it is stated that it has been found that gas-generating charges suitable for a variety of purposes free from disadvantages attendant on the use of hypophosphite or gelatinised nitrocellulose and capable of self-sustained non-detonating decomposition when merely locally heated, with a high yield of hot gases under considerably lower gas pressures than are required for guanidine nitrate, may be obtained by the use in admixture with guanidine nitrate of a polynitrophenol or a polynitrosophenol. Thus co-pending British specification No. 644,073 claims inter alia gas-generating charges comprising guanidine nitrate in admixture with a polynitrophenol or a polynitrosophenol. These charges may include if desired an aliphatic carboxylic acid selected from the group consisting of tartaric, maleic, citric and fumaric acids with or without the inclusion of a small proportion of vanadium pentoxide which if desired may be in the form of a chemically equivalent vanadium compound. These charges may also include a small percentage of a heat resisting material having a large surface area and amounting to not less than 0.25% of the weight of the charge. Furthermore these charges may include thermally volatilizable materials, as for example, insect repellants, insecticides, fungicides, bactericides, and other pesticides.

The object of the present invention is to provide solid gas-generating charges of the kind capable of propagating through themselves a self-sustaining exothermic non-detonating gas-evolving decomposition of guanidine nitrate in admixture with at least one solid polyhydroxy organic compound having a ratio of hydroxyl groups to carbon atoms of at least 1 to 2 in the

2

molecule and which is incapable of supporting its combustion in the absence of oxygen.

According to the present invention gas-generating charges comprise guanidine nitrate in intimate admixture with at least one solid organic polyhydroxy compound having a ratio of hydroxyl groups to carbon atoms in the molecule of at least 1 to 2 and which is incapable of supporting its combustion in the absence of oxygen.

In the absence of diluents or heat-absorbing ingredients a proportion of the said organic compounds amounting to about 5 to 25 per cent of the weight of the guanidine nitrate suffices to render the composition capable of self-sustained decomposition when locally heated, under atmospheric pressure conditions or under conditions of slightly elevated pressure.

It is an advantage of the invention that the compositions may be made by simple admixture of the ingredients, and that when the charge is required to be of compact structure and predetermined form so that it will react only on its exposed external surface it may be made by compressing the mixture into a mould of the desired shape. Moreover, if it is required to protect a portion of the surface of the compact charge from the hot gases evolved by means of an adherent covering of heat-insulating material, this may if desired be done in the course of the pressing operation instead of applying protective material to the surface of the charge after it has been shaped.

When charges made up from guanidine nitrate and a solid organic compound of the aforesaid kind are consumed under atmospheric pressure conditions or at comparatively low super-atmospheric working pressures for example up to about 10 atmospheres, their decomposition into gaseous products is not quite complete, and they leave a certain amount (usually 15 to 20%), of the difficultly fusible nitrogenous organic residue already referred to.

We have found however that the inclusion of a proportion of vanadium pentoxide in a quantity insufficient in the absence of said solid organic polyhydroxy compound to support the self-sustained thermal decomposition at atmospheric pressure of said gas-generating charges, amounting for example to about 0.2 to 1 per cent of the weight of the guanidine nitrate, has the effect in most cases of completing the decomposition of the guanidine nitrate thus obviating the formation of the aforesaid yellow difficultly fusible organic residue and correspondingly increasing the yield of hot gases at working pressures at which this residue would otherwise be formed; and we preferably include in the charge such a proportion of vanadium pentoxide or the equivalent proportion of a chemically equivalent vanadium compound e. g. ammonium vanadate.

It has also been found that a compound of molybdenum e. g. molybdic acid may be used in place of a vanadium compound.

At comparatively low super-atmospheric pressure and under the above conditions the gases contain appreciable quantities of vaporized condensable organic materials, the presence of which may be undesirable in certain applications of the charges, e. g. if they are to be used in driving engines or operating other mechanical devices where these organic vapours can condense and cause fouling of pipes or moving parts.

We have further found that the condensable vaporized organic compounds that would otherwise be formed at pressures near atmospheric

may be destroyed as a result of an exothermic reaction further increasing the hot gas yield, by causing the mixture of gases and vapours, before cooling takes place, to pass over or through suitable heat resisting catalytic solid surfaces such as asbestos or fine wire gauze of iron, steel or platinum, or including in the composition of the charge a small percentage of asbestos fibre or other heat resisting material characterised by a large surface and amounting to not less than about 0.25% of the weight of the charge. The large surface material also steadies the self-supporting characteristics of the reaction and holds together the ash of the charge. It may be desirable to include a small percentage of potassium nitrate in the charge, amounting, for instance, to about 0.25% to 1%, since the potassium nitrate assists the reaction between the gases and vapours on the solid catalytic surface.

Charges made in accordance with the invention may be used for instance for actuating gas pressure operated mechanical devices e. g. for driving engines, or for operating pneumatic tools, for operating fire extinguishers, for propulsion of rockets and other gas escape reaction propelled devices, for dispersing insecticidal or the like substances, for making coloured smokes, or for safety blasting operations by means of blasting assemblies in which the charge is caused to undergo decomposition in a pressure resisting container adapted to vent the gas once a predetermined pressure has been built up within the container. It will be understood that according to the purpose for which the charge is required it may be in powder, granular or compact form of any required shape and may or may not include ingredients for reducing or raising the temperature of the gases it generates. The herein-after mentioned thermally volatilizable materials are examples of ingredients which reduce the temperature of the said gases and by way of example ammonium perchlorate and ammonium nitrate are reagents which raise the temperature of the said gases.

Charges in accordance with the invention may include thermally volatilizable materials, which may be for instance, insect repellents; insecticides, fungicides, bactericides and other pesticides; smoke producing compounds or coloured dyestuffs. In this case the charge will usually be required to decompose under atmospheric pressure conditions; and if the material is an organic compound it will be understood that if the charge is to include asbestos fibre or other material of large surface characteristics its composition must be such that the gases and vapours will not undergo to any extent a reaction on its surface that would destroy the volatilizable compound in the gas stream. The volatilization of the organic compound has a cooling action so that if sufficient of this composition is used the temperature will be too low for any such undesired surface reaction to take place.

The invention is further illustrated by the following examples in which the parts are parts by weight.

#### Example I

A mixture of the following composition:

|                   | Parts |
|-------------------|-------|
| Guanidine nitrate | 80    |
| Tartaric acid     | 20    |

is mixed by milling in a steel ball mill until an intimate and homogeneous powder is obtained. 5 lbs. are then loaded in 3 increments into a 4.7" diameter steel tube closed at one end and lined

with compressed asbestos sheeting, each increment being pressed, under a load of 5,500 lbs./sq. in. A small quantity of incendiary material is placed on top of the charge and the tube is then closed by a screw-on cap in the centre of which is a nozzle 0.128" in diameter. On igniting the incendiary material by an electrical system, self-sustaining decomposition of the charge is induced and continued for 95 secs. maintaining a mean gas pressure in the tube of 300 lbs./sq. in. In this way the charge provides a useful supply of hot gas under pressure suitable for the operation of mechanical devices. A small amount (less than 1 oz.) of a dark brown carbonaceous slag is left in the charge tube after the test.

*Example II*

Glucose and sucrose can each make guanidine nitrate capable of self-sustained decomposition. An intimate mixture is prepared from the powdered ingredients guanidine nitrate and glucose or sucrose in the proportions 90 parts of guanidine nitrate and 10 parts of glucose or sucrose. The mixture is pressed into pellets about 2 cm. diameter and 1½ cm. long. One surface of a pellet is then ignited by means of a flame. The pellet decomposes smoothly in a self-sustained manner giving off copious volumes of gas without showing flame or incandescence. Some yellow infusible residue is left behind.

I claim:

1. Gas generating charges capable, upon local

ignition, of self-sustaining exothermic non-detonating gas evolving decomposition comprising a preponderating amount of guanidine nitrate in intimate admixture with at least one solid organic polyhydroxy compound selected from the group consisting of tartaric acid, glucose and sucrose.

2. Gas generating charges as claimed in claim 1 wherein the proportion of the said organic compounds amounts to 5 to 25% of the weight of the guanidine nitrate in the absence of diluents and heat absorbing ingredients.

3. Gas generating charges capable, upon local ignition, of self-sustaining exothermic non-detonating gas evolving decomposition comprising a preponderating amount of guanidine nitrate in intimate admixture with tartaric acid wherein a portion of the surface of the compact charge is protected by an adherent covering of heat insulating material.

4. Gas generating charges as claimed in claim 3 wherein the heat insulating material is asbestos fibre.

25 References Cited in the file of this patent

UNITED STATES PATENTS

| Number    | Name | Date          |
|-----------|------|---------------|
| 2,165,263 | Holm | July 11, 1939 |
| 2,470,082 | Tyre | May 10, 1949  |